

[54] PROCESS FOR CREATING DESIGNS ON MARBLE

[75] Inventor: David W. Donoho, Baltimore, Md.

[73] Assignee: Hilgartner Natural Stone Company, Inc., Baltimore, Md.

[22] Filed: Oct. 2, 1972

[21] Appl. No.: 294,191

[52] U.S. Cl. .... 156/2, 252/79.2

[51] Int. Cl. .... B44c 1/22

[58] Field of Search .... 156/2, 4, 5, 7, 8, 14, 156/18; 252/79.2

[56] References Cited

UNITED STATES PATENTS

|           |         |           |               |
|-----------|---------|-----------|---------------|
| 1,081,290 | 12/1913 | Albert    | ..... 156/7   |
| 1,313,233 | 8/1919  | Grass     | ..... 156/5 X |
| 1,775,384 | 9/1930  | Beriau    | ..... 156/8   |
| 1,977,372 | 10/1934 | Beriau    | ..... 156/7 X |
| 2,828,192 | 3/1958  | Langsfeld | ..... 156/5   |

|           |         |                |              |
|-----------|---------|----------------|--------------|
| 3,383,254 | 5/1968  | Kocsuta        | ..... 156/5  |
| 3,483,049 | 12/1969 | Grubbe         | ..... 156/5  |
| 3,677,848 | 7/1972  | Stoller et al. | ..... 156/17 |

Primary Examiner—William A. Powell  
Attorney, Agent, or Firm—Roylance, Abrams, Berdo & Kaul

[57] ABSTRACT

There is disclosed a process for creating either a stippled or a striated effect on the surface of a piece of marble. The piece of marble is placed in an acidic solution and positioned so that the exposed surface of the slab faces downwardly. Gas bubbles which are evolved during the action of the acid on the slab remain in controlled contact with the exposed surface of the slab. When the exposed surface is placed facing down in a horizontal position, an eggshell effect is obtained and when the face of the surface is placed down and at an angle, a striated effect is obtained.

10 Claims, 6 Drawing Figures



PATENTED DEC 10 1974

3,853,647

FIG. 1



FIG. 2



FIG. 3



FIG. 4



FIG. 6



## PROCESS FOR CREATING DESIGNS ON MARBLE

This invention relates to a process for imparting a design to the surface of a piece of limestone, and, more particularly, to the surface of a marble slab.

It is known that marble, which is a compact, granular, partly crystallized form of limestone, may be etched by immersing it in an acidic solution. Thus, U.S. Pat. No. 1,977,372 discloses that a printing plate may be made by etching a marble block or slab in an acid solution. The bottom and sides of the marble slab are protected during the etching by a coating of an acid resisting material, the top surface being exposed. During the etching process, various colored parts of the surface of the marble slab are etched at different rates than other colored portions. This selective etching results in a surface having raised portions thereon.

It is an object of the present invention to provide an improved process for creating a decorative effect on the surface of a piece of a limestone.

It is another object of this invention to provide a process for creating an eggshell or stippled effect on the surface of a marble slab.

It is a further object of this invention to provide a process for creating a lined or striated effect on the surface of a marble slab.

These and other objects are accomplished by the practice of this invention, which, briefly, comprises providing a process whereby a piece of limestone, e.g., a marble slab, is positioned in an acidic solution so that gas bubbles which are evolved during the action of the acid on the slab remain in controlled contact with an exposed surface of the slab. This is accomplished by positioning the exposed surface of the slab so that it does not face upwardly — i.e., the exposed surface is placed down either in a horizontal position or at an angle. When the exposed surface is placed facing down in a horizontal position, a stippled effect is obtained, and if the face of the surface is placed down and at an angle, a lined or striated effect is obtained.

The invention will be more particularly described by reference to the accompanying drawings in which:

FIG. 1 is a semi-diagrammatic view illustrating the treatment of a piece of marble according to one embodiment of the invention, the slab of marble being illustrated in side elevation;

FIG. 2 is a plan elevational view of the treated surface of the slab of marble showing the surface after treatment according to the method depicted in FIG. 1;

FIG. 3 is a fragmentary sectional view taken generally on line 3—3 of FIG. 2;

FIG. 4 is a view similar to FIG. 1 illustrating the treatment of a slab of marble according to another embodiment of the invention;

FIG. 5 is a plan elevational view of the treated surface of the marble slab after treatment according to the method depicted in FIG. 4; and

FIG. 6 is a fragmentary sectional view taken generally on line 6—6 of FIG. 5.

In accordance with the practice of this invention, a marble stone or slab is placed in a solution of acid. The face of the slab must always be in the proper position in relation to the surface of the solution, since the angle of the stone in the solution determines the type of finish obtained. For best results, the stone should be flat and smooth. The degree of roughness on the surface of the

stone affects the time required to produce a given finish. The acid in the solution may be hydrochloric acid, nitric acid, phosphoric acid or any other acid having a dissociation constant or ionization constant sufficiently high to etch marble.

Referring specifically to FIG. 1, a marble slab 12 is positioned in the acidic solution 11 and is held off the bottom of the tank 10 by means not shown. For example, the slab may be secured by supporting means attached to the top surface or it may be supported from underneath by a means which will allow circulation of the acid which will permit the acid solution to contact the exposed surface. The exposed surface should be kept off the bottom of the tank 10. The slab 12 is positioned at an angle so that the exposed surface 13 is at an angle of about 45°, as measured from the horizontal, and faces down. The upper surface of the slab and the ends of the slab are protected by a coating of an acid-resisting material 14. The acid solution 11 reacts with the exposed surface 13 resulting in the evolution of gas bubbles 15. Since the marble slab contains areas of varying color, the lighter colored portions are etched at a faster rate than the darker colored portions, thus resulting in a surface having raised portions 16 thereon as shown in FIGS. 2 and 3. The gas bubbles 15 which are evolved during the etching reaction seek to rise to the top of the acid solution 11. However, the bubbles 15 are not free to rise straight to the top from the point at which they are formed since they are in contact with and covered by the surface 13. Accordingly, the bubbles 15 move upwardly along the slanted surface 13 until they reach the upper end 13a at which point they leave contact with the surface and rise straight to the top of the acid solution 11 and escape to the surface at which point they may be disposed of by conventional means.

During the etching process, the acid solution which is in contact with the surface 13 deteriorates — i.e., it becomes weaker due to being neutralized and loses its ability to etch the stone. As the gas bubbles 15 move upwardly along the surface 13 in straight parallel lines, they move away the deteriorated acid solution directly in their path and this deteriorated acid solution is replaced by fresh or undeteriorated acid solution. Since fresh acid solution fills in behind the rising gas bubbles, the etching action in the path of the rising bubbles is more pronounced than in the adjacent areas which remain in contact with deteriorated acid solution. This results in the path of the gas bubbles being etched to a greater extent than the adjacent areas, thereby creating lines or grooves 18 on the surface 13.

The width of the lines or grooves 18 will depend largely upon the angle of the stone in the acid solution 11 during the etching process. Thus, if the stone is placed at an angle of from 80° to 85° from vertical (at an angle of 0° the stone is vertical and at an angle of 90° it is horizontal), relatively wide lines will be obtained whereas relatively fine lines will be obtained when the stone is placed at an angle of from 30° to 45°. In order to obtain more uniform widths of the lines from top to bottom, the position of the stone may be reversed halfway through the etching process so that the relative positions of ends 13a and 13b as shown in FIG. 1 will be reversed.

An auxiliary source of gas bubbles may be provided to cause more bubbles to sweep upward along the surface 13 in order to reduce the time required to obtain

the desired effect. Limestone chips may be placed under the bottom of the slab 12. The action of the acid solution 11 on the limestone chips will create additional gas bubbles. Alternatively, air may be injected into the tank 10 under the bottom of the slab 12, resulting in air bubbles.

If it is desired to lessen the effect of the gas bubbles on the exposed surface of the stone, a gas suppressor such as gum arabic or methyl cellulose may be added to the acid solution. The gas suppressor increases the viscosity of the solution, thereby impeding the movement of the gas bubbles.

The final finish on the stone is affected by the acid content of the solution, the ratio of the volume of the solution to the surface area of the stone, the duration of immersion of the stone in the acid solution, the position of the stone in the acid solution and the composition of the stone.

As shown in FIG. 4, a marble slab 20 of uniform white color is supported by means not shown in a horizontal position (90°) in the acid solution 11. All surfaces of the slab are exposed to the acid solution. Gas bubbles 15 which are evolved during the reaction of the acid solution on marble are free to rise to the surface of the acid solution from the top and edges of the slab. However, gas bubbles 15 which are formed on the underneath surface 21 are trapped against this surface for a time sufficient to cause a large number of very small, localized areas of higher etching action. This results in the production of stippling 22 on the surface 21.

Marble which has been treated by the process of this invention may be used wherever a panel having a decorative effect is desired such as on the walls of buildings.

The following examples illustrate embodiments of this invention:

#### EXAMPLE 1

A marble slab is placed in an acidic solution containing 32 parts of water per part of concentrated (57%) nitric acid. The stone is positioned at an angle of about 45° with the exposed surface facing down and above the bottom of the tank. The ends and the upper surface of the stone are masked with an acid resistant material. A continual stream of gas bubbles is observed to rise to the top of the acid solution from a point directly over the upper end of the slab. After about 20 minutes, the position of the slab is reversed so that the edge which was at the top is at the bottom, the exposed surface of the stone still being kept face down. After about an-

40  
45  
50

other 20 minutes, the stone is removed, washed with water and polished by placing in a dilute acid solution. The exposed surface of the treated stone contains a plurality of longitudinal grooves which give it a lined or striated effect.

#### EXAMPLE 2

A piece of white marble is immersed in an acid solution as described in Example 1. The stone is positioned at an angle of 90° — i.e., it is placed in a horizontal position so that the underside of the stone is exposed to the acid solution. Gas bubbles are observed to rise from around all four edges of the stone. After about 45 minutes, the stone is removed and washed with water. The bottom surface of the stone has a stippled appearance.

I claim:

1. A process for creating a design on a piece of limestone which comprises positioning said piece of limestone in an acidic solution so that the exposed surface of the piece faces downwardly and the gas bubbles which are evolved due to the reaction of the acid with the slab remain in controlled contact with the exposed surface of said slab.
2. A process as defined in claim 1 wherein said piece of limestone is a slab of marble.
3. A process as defined in claim 2 wherein an exposed surface of said slab of marble faces down and is in a horizontal position whereby a stippled effect is obtained.
4. A process as defined in claim 2 wherein an exposed surface of said slab of marble faces down and is at an angle whereby a striated effect is obtained.
5. A process as defined in claim 4 wherein said exposed surface is at an angle of about 45°.
6. A process as defined in claim 4 wherein said exposed surface is at an angle of from about 75° to 85°.
7. A process as defined in claim 4 wherein said exposed surface is at an angle of from about 30° to 40°.
8. A process as defined in claim 4 wherein the position of said slab of marble is reversed about halfway through the process.
9. A process as defined in claim 2 wherein an auxiliary source of gas bubbles is provided.
10. A process as defined in claim 2 wherein a gas suppressor is added to said acidic solution.

\* \* \* \* \*